

# UNITED STATES PATENT OFFICE.

ALBERT C. HOLZAPFEL AND PAUL WALThER, OF NEW YORK, N. Y.

## COMPOSITION FOR COATING NEW IRON AND STEEL.

1,328,282.

Specification of Letters Patent. Patented Jan. 20, 1920.

No Drawing.

Application filed November 13, 1918. Serial No. 262,369.

*To all whom it may concern:*

Be it known that we, ALBERT C. HOLZAPFEL and PAUL WALThER, subjects of the King of Great Britain, residing at New York, in the county of New York and State of New York, have invented certain new and useful Improvements in Compositions for Coating New Iron and Steel, of which the following is a specification.

10 Our invention relates to a composition of matter adapted for coating new iron and steel, and which may be subsequently covered with a paint of a lighter color, while not necessarily restricted to this use.

15 An important object of our invention is to provide a composition of matter of the above mentioned character, which will firmly adhere to the new iron or steel, when applied thereto, and which is insoluble in 20 the paint of lighter color, applied thereto.

Other objects and advantages of the invention will be apparent during the course of the following description.

It is well known that bituminous solutions are adapted to more firmly adhere to new iron and steel, when applied thereto, than ordinary oil paints. This bituminous solution ordinarily contains asphaltum and coal tar pitch, dissolved in hydrocarbons.

30 Owing to the black color of this bituminous solution, it is customary, after the same has suitably dried upon the iron or steel, to coat the same with a paint of a lighter color, thus rendering the material more attractive in 35 appearance. A marked disadvantage encountered in connection with the use of bituminous solutions, as above indicated, is that after drying, they are dissolved by the lighter colored oil paints applied thereto, 40 whereby the lighter colored paints are discolored. Owing to this disadvantage, the bituminous solutions are undesirable for many purposes for which they would otherwise be used.

45 In accordance with our invention, we provide a composition of matter, possessing all of the advantages of the ordinary bituminous solution, but being free from their objections. Our improved composition of 50 matter comprises the following ingredients;

preferably combined in the proportion indicated:

12 parts by weight of stearin pitch,  
20 parts by weight of asphaltum, and  
68 parts by weight of tar oil.

55

The proportion of the asphaltum to the stearin pitch may be reduced or increased according to the qualities of either or both materials, the principal feature of the invention being the use of stearin pitch to render 60 the composition insoluble by the light colored oil paints, when applied thereto.

The composition produced as above indicated is in the form of a bituminous varnish or solution possessing all of the adhesive 65 and protective properties of the usual bituminous or bitumastic solutions, but is not dissolved by ordinary oil paints, which may be subsequently applied to the same so that the oil paints of light color can be readily 70 applied without discoloration.

It is to be understood that the form of our invention herewith described, is to be taken as a preferred example of the same and that various changes may be resorted to in the 75 proportion of the several ingredients and that known chemical equivalents may be employed without departing from the spirit of the invention or the scope of the subjoined claims.

80

Having thus described our invention, we claim:

1. A bituminous varnish or solution for coating iron and steel, comprising tar oils combined with stearin pitch and asphaltum, 85 the combined volume of the stearin pitch and asphaltum being less than the volume of the tar oils.

2. A bituminous varnish or solution for coating iron and steel, comprising approxi- 90 mately 12 parts by weight of stearin pitch, 20 parts by weight of asphaltum, and 68 parts by weight of tar oil.

In testimony whereof we affix our signatures in presence of two witnesses.

ALBERT C. HOLZAPFEL.  
PAUL WALThER.

Witnesses:

MICHAEL DANNOTT,  
MARGARET HOLZAPFEL.